

# UNITED STATES PATENT OFFICE.

EDMUND N. TODD, OF MILBURN, AND WILLIS R. KING, OF NEWARK, NEW JERSEY,  
ASSIGNORS TO THE HANSON & VAN WINKLE COMPANY, OF NEWARK, NEW JER-  
SEY, A CORPORATION OF NEW JERSEY.

## NICKEL-PLATING.

1,352,328.

Specification of Letters Patent. Patented Sept. 7, 1920.

No Drawing. Application filed December 28, 1914, Serial No. 879,312. Renewed February 12, 1920.  
Serial No. 358,127.

*To all whom it may concern:*

Be it known that we, EDMUND N. Todd and WILLIS R. KING, both citizens of the United States, residing at Milburn, in the county of Essex and State of New Jersey, and Newark, in the county of Essex and State of New Jersey, respectively, have invented certain new and useful Improvements in Nickel-Plating, of which the following is a full and clear specification.

Our invention relates in general to the electro-deposition of nickel and contemplates certain improvements in the bath and the process of electro plating, as well as certain improved qualities in the character of the deposit.

In the electro-deposition of metals, many expedients are employed, such as the addition of special agents to the bath, special adjustment of current densities and other electrical relations and special manipulation of the cathode, to secure a certain character of deposit or to achieve some improvement in the process of electroplating. In many cases the theory underlying these special operations or conditions is not understood, but those skilled in the art apply them successfully. In the art of nickel plating, there have been many attempts to secure improvements in the structure and surface characteristics of the deposit, and to reduce the time required for a given thickness of the plating. It has also been sought to increase the thickness of uniform deposit possible, which under the present known methods is quite limited. Beyond a given thickness, the surface becomes irregular and increasingly so as the deposit is continued. A further disadvantage in the nickel plating as practised is the requirement of buffing the plated surface to secure the bright, mirror-like polish which is desired. This buffing process requires the previous deposit of an excess of the metal to allow for loss in buffing, and the buffing operation itself involves a considerable item of time and expense which has heretofore been unavoidable. Furthermore, the buffing is extremely difficult in cases of heavy relief surface, inaccessible to the buffing material.

Our invention has for its object to reduce

the time required for electroplating nickel, to reduce the voltage necessary, to enable the deposit of a substantially uniform deposit of much greater thickness than heretofore possible, and to gain certain important improvements in the internal structure of the deposit as well as certain improvements in the surface characteristics of the deposited metal.

In practising our invention we proceed upon the assumed theory that polarization has an important bearing upon the plating operation and upon the character of the deposit obtained. In the case of a magnetic metal, such as nickel, we assume that the magnetic lines of force proceeding from the polarized cathode cause an unsatisfactory disposition of the nickel ions as they arrive upon the cathode surface, which disposition results in a tendency of the metal to stand out from the cathode and build up a structure which is therefore in adhesion with the cathode surface only at minute points. Furthermore, our theory assumes that under the ordinary practice with a polarized cathode the particles of metal rapidly build outward upon the multiplicity of minute projections due to the repelling influence of the polarization, and contact with each other with only sufficient surface to discharge their charges of current, so that the resulting deposit is not dense and compact. This theory of the effect of polarization upon a magnetic material being deposited would also appear to explain the rapid growth of irregularities upon the surface under ordinary plating conditions which imposes a limit upon the permissible thickness of the coating. According to our theory of operation, the polarization of the electrode is greatly reduced, if not altogether eliminated, and the result is that the particles of the magnetic material are now not repelled by the magnetic lines of force from the cathode and are able to attach themselves closely and compactly to the cathode and to themselves, so that an extremely hard, dense and compact mass of deposit is the result. Furthermore the outer surface is flatter and not broken up by the minute spaces between laterally adjacent particles, so that an even smooth and

mirror-like surface, free from perceptible granulation or facets and having the appearance of fused metal is maintained from the begining right straight through to the conclusion of the electroplating operation. This mirror-like surface maintains an exceedingly uniform exposure of cathode surface to the ions with consequent uniformity of current density and distribution of metal as the deposit grows. The tendency to produce minute outstanding projections being thus minimized the plating is enabled to continue for an almost indefinite period without the objectionable appearance of warts, and other irregularities in the surface. Not only is an extremely hard, dense structure of metal secured, but at the same time an astonishingly smooth and mirror-like surface is obtained, which is even superior to that obtained by the usual buffing operation, which in this case is thus unnecessary. The operation of the plating proceeds much more rapidly and requires lower voltage than under ordinary conditions. The deposit follows exactly the configuration of the cathode upon which it is laid and even the deepest depressions in a heavy relief design are always smooth and highly polished, as though having been subjected to the finest possible buffing. This mirror-like surface is microscopic in its structure, as even a frosted surface when subjected to the plating operation under our invention is reproduced with the same mirror-like gloss. The metal of the deposit displays much higher mechanical strength and tenacity than that obtained by the ordinary plating, and no matter where a fracture is made, the cleavage surface itself presents the same mirror-like character.

The polarization according to the theory assumed by us, is reduced or eliminated by the use of an addition agent in the bath. While, of course, there may be other specific re-agents which will operate under the principles of our invention and produce the desired results, we may mention, as an example, one which has given highly satisfactory results in practice and which may, therefore, be regarded as a representative of a class of materials suitable for this purpose. The substance which we have reference to is contained in the material known in the market as gum tragacanth and while we are aware that this material contains soluble and insoluble substances of which the soluble portion possesses the desired substance for the correction of polarization, we find it not worth while to separate the ingredient but usually employ the gum tragacanth itself without previous separation, and herein designate the agent as gum tragacanth without meaning thereby to limit the invention to the use of the entire substance. It is also to be understood that the invention is not

limited to this specific example, of the agent employed as any other substance performing the same functions will, of course, be embraced within the broad scope of our invention.

With regard to the manner in which the gum tragacanth effects the reduction or elimination of polarization it is, of course, unnecessary to make exact determination, as we believe it to be broadly new to utilize a polarization corrective in connection with the electrodeposition of a magnetic metal in the manner and for the purposes herein described. We may state, however, that in practice we find that the use of gum tragacanth results in the reduction or elimination of the adhesion of hydrogen bubbles to the cathode surface. This fact alone, may, in itself, account for the improvements obtained, under the theory that the adhesion of hydrogen bubbles to the cathode causes the polarization; or the absence of mechanical obstruction caused by the hydrogen bubbles may itself explain the improvements noted. It may be that the result is due in part to each of the conditions. The fact remains that when the gum tragacanth is used in the bath we gain a hard, dense, firmly coherent and homogeneous coating with bright, mirror-like surface, and find that the plating goes faster and requires less voltage. Another peculiar fact is that when the gum tragacanth is employed current densities well in excess of those usually considered permissible can be employed without burning the deposit, resulting in an increased deposit with a lower voltage. The mechanical strength of the deposit is better when low voltage is employed. The same material used as an addition agent to an electroplating bath for non-magnetic metals does not appear to have the same effect as when used in connection with the plating of magnetic metals, such as nickel.

We may state, as an example of a nickel plating bath according to our invention the following: 12 ounces of sulfate of nickel and ammonium in 1 gallon of water, and for each gallon of this solution, 1/15 ounce of gum tragacanth. It will be understood that the exact proportions are subject to considerable variation without departure from the principles of the invention, and the proportions herein stated are only illustrative.

We claim:

1. An electroplating mixture comprising sulfate of nickel and ammonium and an admixture of gum tragacanth.
2. An electroplating mixture comprising the following ingredients, substantially in the proportions stated: 12 ounces sulfate of nickel and ammonium and 1/15 ounce of gum tragacanth.
3. An electroplating solution comprising the following ingredients in substantially

the proportions stated: 12 ounces sulfate of nickel and ammonium, 1/15 ounce of gum tragacanth and one gallon of water.

4. The process of electrodepositing magnetic metal which comprises passing an electric current through an electrolyte having a composition such as to keep a substantially unpolarized condition at the cathode.

5. The process of electrodepositing magnetic metal which comprises passing an electric current through an electrolyte having a composition such as to keep the cathode free from hydrogen bubbles.

6. An electrodeposit of magnetic metal having a hard, dense, firmly coherent internal structure and a bright mirror-like outer surface resembling that of buffed metal entirely free from perceptible granulation, said properties being independent of the initial surface upon which the deposit is produced.

7. An electrolytical deposit of nickel hav-

ing a hard, dense, firmly coherent internal structure, and a continuous outer surface, free from perceptible granulation, having 25 the appearance of fused metal, said properties being independent of the initial surface upon which the deposit is produced.

8. Electrolytic nickel having the qualifications of great hardness and density, a 30 firmly coherent internal structure, continuity of outer surface, free from perceptible granulation both on the surface and throughout the mass, and having the appearance of fused metal.

EDMUND N. TODD.

Witnesses:

R. B. FOX,  
W. L. D. BEDELL.

WILLIS R. KING.

Witnesses:

S. A. PECKENS,  
R. D. FOSTER.